

L. B. TEBBETTS, 2D.  
PRINTING PLATE.  
APPLICATION FILED JULY 1, 1911.

1,087,561.

Patented Feb. 17, 1914.



Attest

*A. J. McGehee*  
E. B. Hines-

Inventor:  
L. B. Tabbetts 2<sup>ND</sup>  
by *Knight & Cook*  
Atty's.

# UNITED STATES PATENT OFFICE.

LEWIS B. TEBBETTS, 2D, OF ST. LOUIS, MISSOURI.

## PRINTING-PLATE.

1,087,561.

Specification of Letters Patent.

Patented Feb. 17, 1914.

Application filed July 1, 1911. Serial No. 636,518.

*To all whom it may concern:*

Be it known that I, LEWIS B. TEBBETTS, 2d, a citizen of the United States of America, residing in the city of St. Louis and 5 State of Missouri, have invented certain new and useful Improvements in Printing-Plates, of which the following is a full, clear, and exact description.

My invention relates to a printing plate, 10 and it has for its object the production of a metal plate of this kind, less expensive than metal plates heretofore made for the same purpose.

With this object in view, the improvement 15 contemplates a multiple ply metal printing plate comprising a facing layer of an alloy of metals which may be readily and efficiently cut by engraving tools to produce a highly satisfactory printing surface and a 20 metal backing layer for such facing layer that is of less expensive nature than the facing layer, but is capable of performing all of the service required at the back of the engraved portion of the plate, such as the 25 furnishing of the necessary stability, rigidity and stiffness in the plate.

Manufacturers of metal printing plates, such as are intended to be prepared by engraving, have for many years endeavored to 30 produce a satisfactory metal printing plate composition consisting of lead and antimony, but it has been found that when sufficient antimony was included in the composition to render the plates of the desired 35 stiffness, the metal was so brittle as to make it impossible to cut clear, sharp, and well defined lines in engraving operations.

By my improvement, I produce a metal 40 printing plate facing surface embodying the materials mentioned, and which is exactly suited to the engraver's needs, this improvement contemplating the employment of another component part of an alloy, namely: tin, which enters into the composition 45 as the main element, is hardened by the presence of antimony, and the alloy, which would otherwise be too stiff and brittle is softened by the addition of a comparatively small percentage of lead relative to 50 the percentage of tin to render the alloy more ductile than it would be if composed of only tin and antimony.

In order that my invention may be more 55 fully understood I will proceed to describe it with reference to the accompanying drawing which is an edge view of my improved

plate showing the layers thereof marked with their constituent elements.

The facing layer of my printing plate, as most commonly made, is composed of tin, 60 antimony and lead, these elements being used in the following proportions, to-wit: tin, from 60% to 90%; antimony, from 2% to 8%, and lead, from 5% to 30%. In this composition, the tin being of a tough nature and being the principal component in the composition serves to render the facing of the plate tough in nature, the antimony serves as a hardening and stiffening agent, and the lead as a softening agent. By the 65 combination of these elements, I produce a printing plate facing layer having all the essential characteristics necessary to permit the production of clear, sharp, and well defined lines when engraving operations are 70 carried out in such layer, inasmuch as the characteristic toughness of the tin compensates for the brittleness of the antimony, the antimony affords the required hardness and stiffness, and the lead in a minor proportion 75 relative to the tin renders the alloy softer and more ductile so that it may be satisfactorily worked in the operations necessary in engraving a printing plate.

The presence of lead in the facing composition is more particularly desirable in producing a printing plate for use in engraving music printing plates, inasmuch as it is common practice in engraving such plates to stamp the note characters by the use of dies, 80 as distinguished from engraving or cutting the other characters and lines; and it is necessary after the stamping operations to partially return the stamped portions of the plate by pressure exerted at the back of the plate, 85 this pressure being usually applied by hammer blows against the body of the plates. In this connection, it is important that the facing layer of the plate be soft or ductile; hence, the desirability of using lead to furnish softness and ductility in the printing 90 plate facing layer.

The facing layer of my printing plate is laid upon and securely attached to a backing layer composed of lead, antimony and tin, 105 these elements being used in the following proportions, to wit: lead, 80% to 97%; antimony, 1% to 15%; tin, 0% to 19%. In this backing layer composition, lead predominates as the main element, being used as 110 such main element principally by reason of its being less expensive than the other ele-

ments; the antimony is used to stiffen the composition, and the tin to toughen the composition. Neither of the last named elements would be satisfactory if used alone with the lead, for the reason that while the antimony would afford the necessary stiffness in the backing layer, its presence alone with the lead would make the composition too brittle; while the tin, if used alone with the lead, would render the composition tough, but would not afford the necessary stiffness. The importance of using the three elements—lead, antimony, and tin in the backing layer is, therefore, apparent.

15 While I have herein described my improvement as relating particularly to a printing plate, there may be other uses for a plate made in accordance with my invention; and I, therefore, do not desire to be limited to its use for any specific purpose.

I claim:—

1. In a metal plate, a facing layer comprising an alloy of tin, a stiffening agent, and a softening agent, the percentage of tin being in excess of the other components in said facing layer; and a backing layer comprising an alloy of lead, a stiffening agent and a toughening agent, the percentage of lead in said backing layer being in excess of the percentages of the other components in said layer.

2. In a metal plate, a facing layer comprising an alloy of tin, antimony and lead, the percentage of tin in said facing layer being in excess of the antimony and lead

therein, and a backing layer comprising an alloy of lead, antimony and tin, the percentage of lead in said backing layer being in excess of the antimony and tin therein.

3. In a metal plate, a facing layer comprising a facing of alloy of from sixty per cent. to ninety per cent. of tin, from two per cent. to eight per cent. of antimony, and of five per cent. to thirty per cent. of lead; and a backing layer comprising lead, a stiffening agent and a toughening agent, the percentage of lead in said backing layer being in excess of the other components in said backing layer.

4. In a metal plate, a facing layer comprising an alloy of from sixty per cent. to ninety per cent. of tin, from two per cent. to eight per cent. of antimony, and from five per cent. to thirty per cent. of lead; and a backing layer comprising an alloy of from eighty per cent. to ninety per cent. of lead, a stiffening agent and a toughening agent.

5. In a metal plate, a facing layer comprising an alloy of from sixty per cent. to ninety per cent. of tin, from two per cent. to eight per cent. of antimony, and of five per cent. to thirty per cent. of lead, and a backing layer comprising an alloy of from eighty per cent. to ninety-seven per cent. of lead, and the balance of antimony and tin.

LEWIS B. TEBBETTS, 2d.

In the presence of—

A. J. McCUALEY,  
E. B. LINN.